# EUROPEAN PATENT SPECIFICATION

(11) **EP 0 522 161 B1**
(45) Date of publication and mention of the grant of the patent: **15.02.1995**
(21) Application number: 91906425.3
(22) Date of filing: 28.03.1991
(51) Int. Cl.: C23F 11/12

(54) **CORROSION INHIBITOR FOR STEAM AND CONDENSER SYSTEM AND CORROSION INHIBITION METHOD THEREFOR**
KORROSIONSSCHUTZMITTEL UND -VERFAHREN FÜR EIN DAMPF- UND KONDENSATORSYSTEM
INHIBITEUR DE CORROSION POUR LA VAPEUR ET LES SYSTEMES CONDENSEURS, ET PROCEDE ASSOCIE D'INHIBITION DE LA CORROSION

(30) Priority: 30.03.1990 JP 81011/90
(43) Date of publication of application: 13.01.1993
(73) Proprietor: AQUAS CORPORATION, Tokyo 152 (JP)
(72) Inventor: AKAMA, Shunichi, c/o Aquas Corporation, Tsukuba-shi, Ibaragi 300-26 (JP); SASA, Takanobu, c/o Aquas Corporation, Tsukuba-shi, Ibaragi 300-26 (JP); YANAGISAWA, Tokuko, c/o Aquas Corporation, Tokyo 152 (JP)
(74) Representative: Reinhard - Skuhra - Weise & Partner
(86) International application number: JP9100410
(87) International publication number: WO9115612

(56) References cited:
- EP-A- 0 039 130
- JP-A-63 137 184
- US-A- 3 149 037
- DATABASE WPI Section Ch, Week 7521, Derwent Publications Ltd., London, GB; Class B03, AN 75-34803W

## Description

### Field of Invention

The present invention relates to a method of preventing the occurrence of corrosion in pipes and devices of steam and condenser systems and the use of vitamin A or a combination of vitamin A and vitamin E and/or their derivatives as anticorrosive agents.

### Background Art

In steam generating apparatuses, such as boilers and concentration cans, the metal in contact with steam and condensed water may corrode due to feed water-containing oxygen and components of M-alkalinity. Regarding to condenser systems in particular, carbon dioxide generated together with steam in boilers and the like dissolves again in water at condensation of steam, leading to the decrease in pH of condensed water (condensation), which frequently causes severe corrosion of pipes and devices. As the methods to prevent such corrosion, there has been conventionally carried out the chemical process with strong basic-type amines such as morpholine and long-chain aliphatic amines such as octadecyl amine, besides the processes of ion exchange and degassing for the objective to degass carbonate in feed water.

In case that the steam generated in boilers is to be used for food processing and the production process of pharmaceutical agents and for humidification of air conditioning of buildings, a high degree of hygienic safety is required for steam. Some of the amine-type chemical agents described above have got approval of their use as the additives for boilers from US FDA Standards, but the objectives of the utility of generated steam have been limited and the concentration of the agents in steam has also limitation. Additionally, they are not necessarily satisfactory in terms of safety. Hence, even in the case that some concerns about the corrosion of pipes and devices of steam and condenser systems may be present, steam is used without chemical processing, in order to ensure safety.

JP-A-49 058 084 discloses a method for controlling redox reaction with a system obtained by combining one or more compound(s) selected from the group (A) and one or more compound(s) selected from the group (B). Examples for the compounds of group (A) are coenzyme Q, vitamin K₂ and plastoquinones; examples for the compounds of group (B) are ubichromenol, ubichromanol and tocopherol (vitamin E). Vitamin A is not mentioned in this document.

EP 0 039 130 discloses the use of dioxo aromatic compounds as oxygen scavengers in an aqueous medium. Examples for such dioxo aromatic compounds are hydroquinone, benzoquinone, naphthoquinone, catechol, and dihydroxybenzaldehyde. Vitamin A is not mentioned in EP 0 039 130.

US 3,149,037 discloses Vitamin compositions comprising Vitamin A or a combination of Vitamin A and Vitamin E for pharmaceutical use.

### Disclosure of the invention

The present invention is thus to provide an anticorrosive method of steam and condenser systems, capable of providing sufficient ensuring of hygienic safety.

The present inventors have carried out investigations so as to achieve the above objectives, and have found that vitamin A or a combination of vitamin A and vitamin E and/or their derivatives among vitamins as the organic substances inevitable for maintaining normal growth and nutritious state of animals, have anticorrosive effects on steam and condenser systems. That is, the present invention provides the use of vitamin and/or its derivatives or a combination of vitamin A and vitamin E and/or their derivatives as anticorrosive agents for steam and condenser systems, and a method for preventing corrosion in steam and condenser systems, comprising the addition of Vitamin A and/or its derivatives or the addition of a combination of vitamin A and vitamin E and/or their derivatives as anticorrosive agents.

The vitamin A to be used in the present invention is ;
(a) vitamin A compounds including vitamin A₁ (retinol), vitamin A₂, vitamin A₃, etc., or
(b) the derivatives of the vitamin A compounds described above, including vitamin A aliphatic acid ester, vitamin A acid, vitamin A aldehyde, etc., and they may be natural products or synthetic products, or those containing such compounds or derivatives, for example, fatty oil obtained from liver and pyrolus uvula of marine animals.

The vitamin E to be used in the present invention is represented by so-called tocopherol and its analogs, including for example, α-tocopherol, β-tocopherol, γ-tocopherol, δ-tocopherol, α-tocotorienol, β-tocotorienol, γ-tocotorienol, δ-tocotorienol, etc. As in vitamin A, oils containing such compounds, for example, germ oil and soybean oil, may be also included.

These vitamins A and E are those incorporated as nutritious components on daily basis into humans, and are substances in a wide range of general use as supplementary products for nutritious foods or additives for milk products, flour, baby foods, condensed and dried soup stocks, curry roux, confectioneries, etc. Vitamins A and E as such are thoroughly investigated of their safety including the effects on human body, so they can appropriately be used in the case that safety of steam is important as described above.

The anticorrosive mechanism is not clear in accordance with the present invention, but such anticorrosive property of vitamin A cannot be expected from the properties and utilities thereof, and the property is very surprising.

Vitamin A is used singly or in combination with vitamin E, or may be used as a pharmaceutical agent in which these vitamins are blended together. The method of adding vitamin A or the mixture of vitamin A and vitamin E, and the concentration thereof to be added should be appropriately determined, depending on equipment condition and the condition as to how to use, and it is generally preferable to directly inject and add them to the pipes of steam or condenser system. The longer the length of pipes of steam or condenser systems gets, the higher the concentration to be added should be. Vitamins A and E are also sparingly soluble in water, and in case that preliminary dilution of them is advantageous at their addition, they may be dispersed in emulsifiers or diluted with solvents, before adding and using them.

### Brief Description of Drawings

Fig.1 is a figure representing the configuration of a testing apparatus to carry out the anticorrosive method of steam and condenser systems in accordance with the present invention.

### Best Mode of carrying out the Invention

While supplying soft water f of the following water quality to autoclave a where as shown in Fig. 1, steam header b, water cooling type steam condenser c following the header b, and condensed water (condensation) pool d following the condenser c, were communicated together, and thermal electric heater e (conductive heat area 0.67 m²) was immersed in water, operation was effected at a steam pressure of 8 kg f/cm², a steam generation volume of 5.5 kg/h, a blower ratio of 10%, and the water temperature in the condensation water pool d of 70 °C, until the final accumulation of feed water reached 200 ℓ. The decrease in corrosion of a soft steel board of 15 mm x 40 mm x 2 mm, suspended in the condensed water pool d, was measured to calculate the corrosion degree (mdd). Chemical agents g used are as follows, and the agents were injected into the steam header b at their ratios to condensed water as shown in Fig.1. No chemical agents were injected into the autoclave a.

The results are shown as Fig.1, and excellent anticorrosive effect was obtained.

### Quality of soft water

| | |
|---|---|
| pH | 7.5 |
| Electric conductivity (»S/cm) | 200 |
| M-alkalinity (mg CaCO₃) | 48 |
| Silica (mg SiO₂) | 24 |
| Chloride ion (mg Cl/l) | 13 |
| Whole hardness (mg CaCO₃) | less than 1 |

### Chemical agents used

| Chemical agent A: | |
|---|---|
| Vitamin A (Riken A palmitate 1000) | 1 % |
| Benzyl alcohol | 99 % |

| Chemical agent B: | |
|---|---|
| Vitamin A (Riken A palmitate 1000) | 4.1 % |
| Benzyl alcohol | 95.9 % |

| Chemical agent D: | |
|---|---|
| Benzyl alcohol | 100 % |

| Chemical agent E: | |
|---|---|
| Octadecyl amine | 1.4 % |
| Polyoxyethylene stearylether | 0.4 |
| Water | 98.2 % |

| Chemical agent F: | |
|---|---|
| 2-Amino-3-methyl propanol | 17.5 % |
| Water | 82.5 % |

**Table 1**

| Test No. | Chemical agent | Amount added (»g/litre) | Corrosion degree(mdd) | Note |
|---|---|---|---|---|
| 1 | blank | | 125 | |
| 2 | A | 600 | 22 | Example |
| 3 | B | 600 | 34 | Example |
| 5 | D | 600 | 124 | Comparative Example |
| 6 | E | 600 | 41 | Comparative Example |
| 7 | F | 600 | 27 | Comparative Example |

### Industrial Utilization of the Invention

Because an anticorrosive agent containing as the effective component vitamin A or a combination of vitamin A and vitamin E and/or their derivatives is injected into steam pipes or into boilers, the application of the anticorrosive method of steam and condenser systems in accordance with the present invention allows the use of the steam for food processing and the like, with no concerns about the occurrence of steam contamination and the corrosion of the pipes due to chemical agents and the like.

## Claims

1. Use of vitamin A and/or its derivatives or a combination of vitamin A and vitamin E and/or their derivatives as anticorrosive agents.

2. Use according to claim 1 wherein the anticorrosive agents comprise additionally an emulsifier or a solvent.

3. Use according to claim 2 wherein said solvent is a benzyl alcohol.

4. A method for preventing corrosion in steam and condenser systems, comprising the addition of vitamin A and/or its derivatives as anticorrosive agents.

5. A method for preventing corrosion in steam and condenser systems, comprising the addition of a combination of vitamin A and vitamin E and/or their derivatives as anticorrosive agents.

## Patentansprüche

1. Verwendung von Vitamin A und/oder seiner Derivate oder einer Kombination von Vitamin A und Vitamin E und/oder ihrer Derivate als Antikorrosionsmittel.

2. Verwendung nach Anspruch 1, worin die Antikorrosionsmittel zusätzlich einen Emulgator oder ein Lösungsmittel umfassen.

3. Verwendung nach Anspruch 2, worin das Lösungmittel ein Benzylalkohol ist.

4. Korrosionsschutzverfahren in Dampf- und Kondensatorsystemen, umfassend die Zugabe von Vitamin A und/oder seiner Derivate als Antikorrosionsmittel.

5. Korrosionsschutzverfahren in Dampf- und Kondensatorsystemen, umfassend die Zugabe einer Kombination von Vitamin A und Vitamin E und/oder ihrer Derivate als Antikorrosionsmittel.

## Revendications

1. Utilisation de vitamine A et/ou de ses dérivés ou d'une combinaison de vitamine A et de vitamine E et/ou de leurs dérivés comme agents anticorrosifs.

2. Utilisation selon la revendication 1, dans laquelle les agents anticorrosifs comprennent de plus un émulsifiant ou un solvant.

3. Utilisation selon la revendication 2, dans laquelle ledit solvant est l'alcool benzylique.

4. Procédé pour éviter la corrosion dans des systèmes à vapeur et condenseur, comprenant l'addition de vitamine A et/ou de ses dérivés comme agents anticorrosifs.

5. Procédé pour éviter la corrosion dans des systèmes à vapeur et condenseur, comprenant l'addition d'une combinaison de vitamine A et de vitamine E et/ou de leurs dérivés comme agents anticorrosifs.
